

## UNITED STATES PATENT OFFICE

2,081,828

## IMPREGNATING WOOD

Frank H. Lyons, Memphis, Tenn., assignor to  
E. L. Bruce Co., Memphis, Tenn., a corporation  
of Delaware

No Drawing. Application January 20, 1930,  
Serial No. 422,223. Renewed October 2, 1936

## 5 Claims. (Cl. 21—52)

My invention relates to the impregnating of wood and the like and has particularly in view the treatment of lumber so that it will resist insect and fungi attack, such as from termites and rot fungi.

Various processes having in view the same purpose have been utilized heretofore, but have as a rule some insufficiency. Creosoting the wood is not satisfactory on account of the odor of the creosote. Zinc chloride, zinc meta-arsenite, Wolman salts and similar preservatives, must be applied to the wood in the form of an aqueous solution and according leave the treated lumber with a high moisture content. This necessitates a 15 drying time of from three to six months before the lumber can be used for building operations. Pressure processes which are the kind that are in most common use necessitate the stocking of large quantities of lumber for satisfactory operation.

20 One of the objects of my invention is to provide a process by which it is possible to achieve in a reasonable time, adequate penetration of the wood by a non-water preservative, without 25 objectionable odor, using an open tank process.

Moisture is held in the wood in at least two 30 different ways. One way is by absorption by the cell walls. Another way is the holding of water mechanically on the cell walls i. e. adsorption. Under a standard condition of temperature and pressure, these two forms of moisture retention are in dynamic equilibrium i. e. the adsorbed 35 moisture is changing to absorbed moisture as fast as absorbed moisture is changing to adsorbed. Penetration of an oil into the wood under these conditions by capillary attraction is, from a theoretical standpoint, difficult.

Increased penetration may be had by (1) the 40 addition of a compound to the treat to make the capillary attraction more positive; (2) a preliminary treatment of the wood to make the capillary attraction more positive; and (3) evaporation of the moisture in the wood.

These ends are all attained by treating the 45 wood by my method and with my composition in an open tank. The composition is heated by any suitable means to approximately 240° F. and maintained at this temperature. The wood is immersed in the bath and held there until it has 50 reached practically the temperature of the bath and then it is transferred as quickly as possible to a second bath in which the same composition is at a temperature of approximately 140° F. In the hot bath, the moisture is largely driven 55 out of the wood and the wood is expanded. When

the wood is plunged into the cooler bath, the vacuum, which is created by the condensation of any water vapors in the wood, by the cooling of any air left in the wood, and by the capillary attraction, serves to draw the treat into the wood. 5

The preferred composition that I have discovered and found efficient in use is as follows:

|                       |         |        |
|-----------------------|---------|--------|
| 38-40° Bé. fuel oil   | gallons | 480    |
| 18-20° Bé. fuel oil   | do      | 480    |
| Ortho-dichloro-benzol | pounds  | 109 10 |
| Beta naphthol         | do      | 350    |

These quantities will make up approximately 1000 gallons of treating solution.

The fuel oil acts as a solvent for the beta naphthol which is a toxic material. The ortho-dichloro-benzol increases the penetration of the toxic bearing oil. Other solvents than fuel oil could be employed such as solvent naphtha, benzol, carbon tetrachloride, etc. Other organic 20 toxic materials than beta naphthol could be used such as di-nitro-chloro-benzene.

Other penetration accelerators than ortho-dichloro-benzene can be used such as para-dichloro-benzene.

About 5% of beta naphthol is soluble in the aforesaid composition at 140° F. but at 70° F. 25 50% of the beta-naphthol crystallizes out of solution. For a substance to be toxic, it must be at least slightly soluble in water. Beta naphthol is soluble to the extent of one pound to every thousand pounds of water. The presence of the beta-naphthol in the precipitated form assures conditions such that any water present can dissolve its full amount of beta-naphthol, the solubility 30 35 being low enough to insure a long period of toxicity.

If the beta-naphthol, dissolved to saturation in cold oil, is injected into the wood, the solubility of the beta-naphthol in water from this oil solution would be below the toxic strength desired to kill the fungi, but by using a hot saturated solution of beta-naphthol, there is deposited on cooling, as free crystals, about 50% of the beta-naphthol on the fibers of the wood and this free beta-naphthol is available for saturating any moisture in the wood to a strength much above that required for killing fungi. There is, therefore, available as a fungicide both the toxic dissolved in the oil and the toxic which is present 40 45 50 as free toxic deposited on the fibers of the wood.

By my invention I am able to impregnate wood or the like by a novel method with a toxic substance, which thereafter partially crystallizes along the cell walls.

The operating results of the process in practice will be clear from the following example.

Six hundred and forty board feet of pine timbers 2 in. x 6 in. x 12 ft. weighing about 2,960 lbs. were stacked in a crate so as to allow a one inch space around each timber, and immersed in a tank containing the treating composition heated to 240° F. After remaining for 45 min., the load was removed from the hot tank and immediately submerged in the cold tank, which is kept at 140° F. by means of a steam coil. During the heating period in the hot tank the air in the wood is expanded and some of the moisture is evaporated. As the timbers cool in the cold tank, the air contracts and the water vapors condense and the treating composition is drawn in. Due to the particular composition of the treating solution, more penetration is obtained by capillarity than with the fuel oil alone. The composition being used at 140° F. the 5% by weight of beta-naphthol is entirely in solution. After about 45 minutes the load is removed from the cool tank and weighed. As the lumber cools, the beta-naphthol crystallizes from solution until at 70° F. one-half of the total amount has crystallized. The weight of the timber when taken from the cold tank was 3,210 lbs., about 250 lbs. of treating composition having been absorbed.

From the description, it will be seen, that I provide a toxic material which is soluble in organic solvents, and more soluble at the higher than the lower temperature. I am therefore, able to treat lumber with a solution of a toxic material at an elevated temperature, the solution being saturated at the final treating temperature with the toxic material, which on cooling, deposits the excess toxic on the fibers of the wood. In this way, I am able to impregnate wood without the use of water, with a toxic material which is present in the free state and in the solvents, at the ordinary temperature of the wood.

While I have disclosed my invention in connection with the impregnating of wood, it is obvious that other porous materials could be similarly treated.

I claim:

1. The method of impregnating wood and the like to resist insect and fungi attack, with a solution containing as a toxicant, beta-naphthol or the like in petroleum oil solvents, about 5% of the toxicant being soluble at about 140° F. and 50% crystallizing out at about 70° F., comprising treating the wood with the hot solution to cause substantial impregnation of the wood therewith and lowering the temperature to cause crystallization of the toxicant onto the fibers of the wood.

2. The method of impregnating wood and the like to resist insect and fungi attack, with a solution containing as a toxicant about 5% of beta-naphthol or the like dissolved in petroleum fuel oils at about 140° F., comprising treating the wood with the hot solution to cause substantial impregnation of the wood therewith and lowering the temperature to cause crystallization of the toxicant onto the fibers of the wood, about 50% of the toxicant crystallizing out onto the wood at 70° F., the amount of toxicant precipitated being sufficient to dissolve in any aqueous medium present to a concentration above that required to inhibit the growth of fungi and insect attack. 15

3. The method of impregnating wood and the like to resist insect and fungi attack, with a solution containing beta-naphthol or the like in a petroleum oil solvent made up of a mixture of equal parts of 38-40° Bé. and 18-20° Bé. fuel oils, 20 about 5% of the toxicant being soluble in the oil mixture at about 140° F. and 50% crystallizing out at about 70° F., comprising treating the wood with the hot solution to cause substantial impregnation of the wood therewith and lowering the temperature to cause crystallization of the toxicant onto the fibers of the wood, the amount of toxicant precipitated being sufficient to dissolve in any aqueous medium present to a concentration above that required to inhibit the 25 growth of fungi and insect attack. 30

4. The method of impregnating wood or the like to resist insect and fungi attack with a solution containing as a toxicant, beta-naphthol or the like in a non-volatile oil solvent comprising 35 treating the wood with said solution at an elevated temperature to cause substantial impregnation of the wood with the solution and lowering the temperature to about 70° F. to cause crystallization of a part of the toxicant onto the 40 fibers of the wood, the amount of toxicant dissolved in the said oil at the elevated temperature and the solubility of the toxicant in said oil at the lower temperature being such that the 45 amount of toxicant precipitated is sufficient to dissolve in any aqueous medium present to a concentration above that required to inhibit the growth of fungi and insect attack. 50

5. A wood article of manufacture impregnated with crystallized beta-naphthol and beta-naphthol in a non-volatile oil solvent, the amount of crystallized beta-naphthol being sufficient to dissolve in any aqueous medium present to a concentration above that required to inhibit the 55 growth of fungi and insect attack. 55

FRANK H. LYONS.